

# United States Patent [19]

Weinberger

[11] 4,371,377

[45] Feb. 1, 1983

[54] FUEL ADDITIVE

[75] Inventor: Theodore Weinberger, Charlotte, N.C.

[73] Assignee: Adriel Energy Corporation, McLean, Va.

[21] Appl. No.: 210,601

[22] Filed: Nov. 26, 1980

[51] Int. Cl.<sup>3</sup> ..... C10L 1/02

[52] U.S. Cl. ..... 44/56; 44/77

[58] Field of Search ..... 44/56, 77

[56] References Cited

U.S. PATENT DOCUMENTS

|           |         |         |       |
|-----------|---------|---------|-------|
| 1,399,227 | 12/1921 | Rohrs   | 44/77 |
| 1,423,049 | 7/1922  | Tunison | 44/77 |
| 2,106,662 | 1/1938  | Savage  | 44/56 |

|           |         |         |         |
|-----------|---------|---------|---------|
| 2,143,870 | 1/1939  | Ellis   | 44/9    |
| 2,496,444 | 2/1950  | Cook    | 44/77   |
| 3,511,218 | 5/1970  | Lazaros | 123/119 |
| 3,594,136 | 7/1971  | Rosen   | 44/51   |
| 4,207,076 | 6/1980  | Bove    | 44/56   |
| 4,231,756 | 11/1980 | King    | 44/77   |

Primary Examiner—Charles F. Warren

Assistant Examiner—Y. Harris-Smith

Attorney, Agent, or Firm—Cushman, Darby & Cushman

[57] ABSTRACT

Higher ratios of alcohol to gasoline (gasoline) are possible utilizing gasoline in combination with a mixture of alcohol, a ketone (e.g., acetone) and a small amount of an alkali metal carbonate, such as sodium carbonate, in finely divided form.

13 Claims, No Drawings

## FUEL ADDITIVE

## BACKGROUND OF THE INVENTION

The present invention relates to an improved fuel mixture for internal combustion engines, notably those engines which are powered by gasoline.

With petroleum resources dwindling throughout the world, efforts are constantly being made to utilize alternative sources of energy. Recently, mixtures of gasoline and alcohol (most notably ethanol) have been touted as but one means of an alternate means of saving energy. In order to increase the use of such gasohol products, there is a need for increasing the proportion of alcohol which can be used in such mixtures without a loss in performance or damage to the engine. Current gasohol products contain approximately 10 percent by volume alcohol with the balance being chiefly gasoline together with conventional additives (e.g. combustion catalysts, etc.).

Prior to the recent commercialization of gasohol products, a variety of alternatives to gasoline per se had been suggested for use in internal combustion engines as exemplified in U.S. Pat. Nos. 1,399,227 and 1,423,049. However, the use of gasohol appears to offer the great potential for the reduction of petroleum consumption, particularly if greater proportions of alcohol can be effectively incorporated into the fuel mixture.

Accordingly, it is the primary object of the present invention to provide an additive for gasoline in combination with alcohol which will enable one to fuel an internal combustion engine with larger proportions of alcohol than utilized herebefore.

It is a further object of the present invention is to employ a fuel mixture containing a substantial amount of alcohol and which meets or exceeds both federal and state emission requirements.

These and other objects of the present invention will be more apparent from the discussion which follows hereinafter.

## SUMMARY OF THE INVENTION

The present invention is directed to an admixture which used in combination with various ratios of gasoline and alcohol enables higher proportions of alcohol to be effectively employed without sacrificing performance or damaging the internal combustion engine.

Specifically, the alcohol and additive mixture of the present invention consists essentially of an alcohol and from about 3 to about 10 percent by volume, based on the alcohol of a ketone having the general formula



wherein  $\text{R}_1$  and  $\text{R}_2$ , which may be the same or different, are each an alkyl of 1 to 4 carbon atoms, and from about 0.3 to about 1.5 grams, and preferably 0.36 to 1.2 grams, per gallon of the alcohol and ketone mixture of an alkali metal carbonate in finely divided form.

Currently as noted, alcohol such as methyl alcohol, ethyl alcohol or mixtures thereof is added in an amount of about 10 percent by volume to gasoline mixtures to form a fuel mixture referred to as gasohol. This alcohol is generally at least 190 proof. Alcohols containing greater amounts of moisture heretofor have been considered unsuitable as for use in gasoline mixtures as such

low proof alcohols are inefficient and potentially hazardous to the engine due to their high water content. The addition of a ketone in accordance with the present invention in combination with the finely divided alkali metal carbonate (e.g. in the form of a powder 100 mesh or finer) enables one to utilize not only a greater proportion of alcohol in combination with the gasoline (e.g., up to about 35, 40 or even 50 percent by volume alcohol), but also permits the use of alcohols containing a greater amount of moisture (e.g., as low as 170 proof).

The invention further embodies a fuel additive consisting essentially of a ketone having the general formula



wherein  $\text{R}_1$  and  $\text{R}_2$ , which may be the same or different, are each an alkyl of 1 to 4 carbon atoms and from about 10 to about 15 grams of an alkali metal carbonate in finely divided form per gallon of ketone.

Thus, there is provided in accordance with one embodiment of the present invention a fuel suitable for operating an internal combustion engine which comprises from about 50 to about 95 percent by volume gasoline and from about 50 to 5 percent by volume of the alcohol and additive mixture described hereinabove. Preferably the fuel mixture contains from about 70 to 90 percent by volume gasoline and from about 30 to 10 percent by volume of said alcohol and additive mixture. An especially preferred ratio is 75 percent gasoline and 25 percent alcohol and additive mixture.

A number of advantages flow from the use of the fuel admixtures called for in the present invention. Of particular note is the ease with which an engine will start in cold weather. In addition, the fuel mixture of the present invention burns cleaner and exhibits less carbon deposit than current gasohol or gasoline fuels. The resulting fuel mixture meets or exceeds federal and state emission requirements.

As noted, the alcohol and additive mixture contains from about 3 to about 10 percent based on the weight of the alcohol of a ketone having the formula noted above. While a variety of ketones could be employed, an especially preferred ketone is selected from the group consisting of acetone, methyl-ethyl ketone or mixtures thereof. Acetone is especially preferred due to its ready availability and low cost. The amount of ketone may vary within the range stated and preferably ranges from about 5 to about 7 percent based on the volume of the alcohol.

The alkali metal carbonate most suitable is sodium carbonate, but it is also envisioned that one might employ with equal efficiency potassium carbonate, lithium carbonate or mixtures thereof in a finely divided state. The carbonate must be in a sufficiently fine divided state to readily mix with the alcohol, acetone and gasoline and not clog fuel jets or lines. Thus, powdered particles of at least 100 mesh or finer are preferred. The carbonates serve to enhance the fuel mixture by apparently controlling the amount of water which may be present. Only a small amount of the carbonate need be present and generally from about 0.3 to about 1.5 grams per gallon of the alcohol and ketone mixture need be employed. Preferably one utilizes approximately 0.36 to 1.2 grams of the carbonate per gallon of alcohol and ketone mixture.

An especially preferred fuel mixture according to the present invention comprises:

about 70 to 90% by volume gasoline; and  
about 30 to 10% by volume of an alcohol and additive mixture consisting essentially of:

about 90 to 97 percent by volume ethanol;  
about 10 to 3 percent by volume of a ketone selected from the group consisting of acetone, methyl-ethyl ketone and mixtures thereof; and  
about 0.3 to 1.5 grams of sodium carbonate per gallon 10 of alcohol and ketone mixture.

The presence of the ketone in combination with the alcohol appears to enhance the combustibility of the resulting fuel mixture when admixed with gasoline. The fuel additive may be employed both with unleaded as well as leaded type gasolines currently available on the market.

Insofar as the preparation of the fuel additive or resulting fuel mixture is concerned, there is no criticality in the mode by which the ingredients are blended. Thus, the carbonate may be added directly to the alcohol or mixtures of the alcohol and acetone. Alternatively, the ingredients may be individually, and with no critical order of addition, added to the gasoline within the proportions described.

The following examples are offered in order to more fully illustrate the invention, but are not to be construed as limiting the scope thereof.

#### EXAMPLE 1

A gasoline additive was prepared by thoroughly mixing together the following materials in the amounts indicated:

acetone 1 gallon  
sodium carbonate 12 grams per gallon of acetone in 35 powder form.

#### EXAMPLE 2

The additive of Example 1 was mixed with varying amounts of unleaded regular gasoline and alcohol (190 proof ethanol). The resulting fuel mixture was then tested in a 1979 Dodge Aspen equipped with a 2-barrel carburetor. The tests were carried out at 50 mph. Fuel mileage figures were determined by taking a minimum of five tests and averaging the totals. For purposes of comparison, tests were also run using unleaded regular gas. The results are set forth in Table I.

TABLE I

| Test No. | Volume Gasoline | Volume Alcohol | Additive (oz.) | Miles per gallon | Hydrocarbons ppm | CO % |
|----------|-----------------|----------------|----------------|------------------|------------------|------|
| 1        | 100             | —              | —              | 19.78            | 84               | .56  |
| 2        | 60              | 40             | 8              | 16.66            | 47               | .01  |
| 3        | 70              | 30             | 7              | 17.4             | 73               | .01  |
| 4        | 75              | 25             | 6              | 19.4             | 56               | .02  |

Overall, the results of the foregoing examples demonstrate the unexpected performance of the additive and resulting fuel mixture.

The additive was also found to be effective at both 60 speeds of 35 as well as 55 miles per hour. Additional observations included idling periods and acceleration and deceleration at stop lights, shopping center parking lots, and other specifically designated points.

While certain representative embodiments and details have been shown for the purpose of illustrating the present invention, it will be apparent to those skilled in the art that various changes and modifications may be

made therein without departing from the spirit and scope of the invention. It will further be understood that the invention may comprise, consist essentially of or consist of the steps or materials recited herein.

5 I claim:

1. A gasoline additive mixture consisting essentially of alcohol mixed with from about 3 to about 10 percent, based on the volume of said alcohol, a ketone having the general formula



15 wherein R<sub>1</sub> and R<sub>2</sub>, which may be the same or different, are each an alkyl of 1 to 4 carbon atoms, and from about 0.3 to about 1.5 grams per gallon of said additive mixture of an alkali metal carbonate in finely divided form.

2. The additive of claim 1 wherein said ketone is selected from the group consisting of acetone, methyl-ethyl ketone and mixtures thereof.

3. The additive of claim 1 or 2 wherein said alkali metal carbonate is sodium carbonate.

4. The additive of claim 1 or 2 wherein said ketone is present in an amount ranging from about 5 to about 9 percent based on the volume of said alcohol.

5. The additive of claim 4 wherein said alcohol is methyl alcohol, ethyl alcohol or mixtures thereof.

6. The additive of claim 5 wherein said carbonate is present in an amount ranging from about 0.36 to 1.2 grams per gallon.

7. A fuel additive consisting essentially of a ketone having the general formula:



wherein R<sub>1</sub> and R<sub>2</sub>, which may be the same or different, are each an alkyl of 1 to 4 carbon atoms and from about 10 to about 15 grams of an alkali metal carbonate in finely divided form per gallon of ketone.

8. The additive of claim 7 wherein said ketone is selected from the group consisting of acetone, methyl-ethyl ketone and mixtures thereof.

9. The additive of claim 7 consisting essentially of acetone and about 12 grams of sodium carbonate.

10. A fuel for an internal combustion engine comprising from about 50 to 95 percent by volume gasoline and from about 50 to 5 percent by volume of the additive of claim 1 or 2.

11. The fuel of claim 10 comprising from about 70 to 90 percent by volume gasoline and from about 30 to 10 percent by volume of said additive.

12. The fuel of claim 10 comprising:  
about 70 to 90% by volume gasoline; and  
about 30 to 10% by volume of a gasoline additive mixture consisting essentially of:  
about 90 to 97 percent by volume ethanol;  
about 10 to 3 percent by volume of a ketone selected from the group consisting of acetone, methyl-ethyl ketone and mixtures thereof; and  
about 0.36 to 1.2 grams of sodium carbonate in finely divided form per gallon of additive mixture.

13. A method for fueling an internal combustion engine which comprises feeding to said engine under combustion conditions the fuel of claim 10.

\* \* \* \* \*